

Patented July 20, 1926.

1,592,935

# UNITED STATES PATENT OFFICE.

ELMO G. HICKEY, OF LOS ANGELES, CALIFORNIA.

## PROCESS OF RECOVERING TIN.

No Drawing.

Application filed April 28, 1925. Serial No. 26,524.

This invention relates to process for recovering tin from tin cans, scrap tin and other tin surfaces.

For approximately the past fifty years various processes for the removal of tin from tin bearing scrap, tin cans and the like, have been known and used. These processes have, for the most part, been based upon the fact that tin is soluble in either hot or cold solutions of caustic alkali in the presence of alkali metal nitrates. These processes have, for the most part, a number of difficulties, one of which difficulties has been in the development of this recovery process from the standpoint of commercial success because of the relatively long time required for this action to take place and the consequent excessive high cost in plant expense, handling charges of any considerable quantity of material to be "detinned", such as tin scrap, refuse, tin cans, and the like.

An object of this invention is to provide a process by which the tin may be recovered from tin scrap, refuse, tin cans, and the like, in a relatively short time, maintaining a high efficiency of the recovery of the tin.

I have discovered that the recovery of tin is greatly accelerated by the addition of ammonia to the alkaline solution composed of caustic soda and alkaline nitrates. According to the preferred form of the invention, the tin scrap, tin cans, and the like, properly cleaned and perforated, is subjected to the action of a solution of caustic soda and sodium nitrate to which from 3% to 3% by weight of ammonium hydroxide has been added; the ammonium hydroxide used being approximately 28%  $\text{NH}_3$ . The solution is heated approximately to boiling. This solution is from 4 to 12% sodium nitrate and from 18 to 28% sodium hydroxide, although it is to be understood that other alkali-metal hydroxides might be employed

and that nitrates other than sodium nitrate might be employed in this process with equal efficiency, sodium nitrate and sodium hydroxide being employed because of the ease in which the same can be obtained and the expense of the different chemicals.

By the use of this ammonia, I have discovered that the tin will be completely removed from the tin scrap within approximately an hour, where heretofore it has required from 6 to 7 hours to obtain the same tin recovery.

Having fully described the preferred embodiment of this invention, it is to be understood that this invention relates to the use of ammonia as a catalytic agent for accelerating the rate of recovery of tin from tin scrap and that the same is in no way dependent upon the percentages of sodium hydroxides and sodium nitrate employed other than that the same should be of sufficient strength to remove the tin from the tin bearing scrap and precipitate the same, preferably as sodium stannate.

I claim:

1. A process of recovering tin from tin scraps which comprises subjecting the tin scraps to the action of caustic alkali and alkali metal nitrate in the presence of ammonia.

2. A process of recovering tin from tin scraps comprising subjecting tin scrap to the action of caustic alkali and alkali metal nitrate in the presence of from 3 to 3% of ammonia hydroxide containing 28% ammonia by weight.

3. In a process of recovering tin from tin scraps, employing caustic alkali solution, the step which includes the use of ammonia as an energizing agent.

Signed at Los Angeles, California, this 23d day of April 1925.

ELMO G. HICKEY.